

## UNITED STATES PATENT OFFICE.

HOWARD F. WEISS, OF MADISON, WISCONSIN, ASSIGNOR, BY MESNE ASSIGNMENTS, TO  
C. F. BURGESS LABORATORIES, INC., OF DOVER, DELAWARE, A CORPORATION OF  
DELAWARE.

PARAFFIN-RESISTING SURFACE FOR PARAFFIN-ABSORBENT BOXES AND METHOD OF  
MAKING SAME.

No Drawing.

Application filed May 15, 1925. Serial No. 30,623.

My invention provides a method for coating paper, so that molten paraffin heated to the smoking point, as well as other waxes, greases and oils, will be prevented from 5 reaching the paper and saturating it. This method of preventing the paraffin from saturating the coated paper is of much importance in the manufacture of boxes, such for instance, as are used for radio B-batteries, 10 although it can be applied to other manufacturers.

According to usual practice B-battery boxes are made of a chipboard or similar paper product which has the property of 15 absorbing large quantities of molten paraffin. A suitable label is pasted on the exterior of the chipboard box. The labeled box is then saturated with paraffin heated to smoking which drives out all of the moisture and makes the box thoroughly waterproof. The label, which may be printed on white paper, becomes thoroughly saturated with paraffin and the paper becomes translucent. On the other hand, the chipboard 20 box acquires a dark color when saturated with paraffin so that the translucent white label paper assumes a dirty white color which gives the box an undesirable appearance. Other colors also assume a dirty 25 appearance.

My invention provides a method for coating such labels so that the paraffin cannot penetrate the paper, thereby preserving the desirable clean color of the printed labels.

I have found that if paper is dipped into colloidal solutions (from 3 to 6 percent) of starch, casein, silicate of soda, gelatine, glue, collodion, etc., a film is formed on the paper, which, after drying, prevents paraffin, which has been heated to smoking, from reaching the paper, except for occasional pinholes. The effectiveness of the protecting film is determined by the number of pin holes. The films formed by these 40 various colloidal solutions have the defect of being brittle. The fragile nature of the film does not allow the paper to be roughly handled and the film is likely to be ruptured or cracked during subsequent manipulation. These cracks allow the paraffin to 45 penetrate to the paper. I have discovered

further that this brittleness may be overcome by adding a non-drying material to the glue or other coating solutions. This non-drying material tempers the film and 55 keeps it flexible. Glycerine, rubber latex, and dextrose are examples of materials which may be added to the coating solution.

It is desirable to print labels, which are to be paraffined, after the paper is coated 60 with the paraffin-resisting film. If the film does not contain the non-drying fluid, the printing operation ruptures the film on the surface. I have discovered that paper coated with a film of a suitable paraffin-resisting 65 material, such as sizing glue, to which glycerine has been added, may be put through the printing press without rupturing the film. A water solution containing 6 per cent of sizing glue and 3 per cent of glycerine 70 gives excellent results.

It has not been found necessary to coat both sides of labels which are to be pasted onto a backing material, such as B-battery boxes. If a suitable adhesive, such as box- 75 factory glue, is used to paste the label onto the box, this adhesive, if heavy enough, acts as a film which prevents the paraffin from penetrating the label during saturation of the absorbent box.

While my invention has its special application in the labeling and paraffining of B-battery boxes, it can be used wherever a paraffin-resistant paper surfacing is required. I define "paraffin-resistant" as excluding all paraffin. There are papers which absorb but small quantities of oils, greases, waxes or paraffin, but such papers are not suitable as labels for B-battery boxes and are not included under my definition of 85 "paraffin-resistant."

Although the claims refer to molten paraffin, I do not wish to be limited to this material since my invention is also applicable to paper made resistant to waxes, oils and 95 greases.

In the manufacture of B-battery boxes, the labels are first coated on one or both sides with a paraffin-resisting film, the labels are then printed over this film, after which 100 they are pasted onto the chipboard box, box-factory glue being used if the reverse

side of the label has not been protected with a film, following which the finished box is ready for the paraffining operation.

I claim:

5. 1. The method which consists in coating at least one side of a sheet of paper with a paraffin-resisting colloid, pasting said sheet to a paraffin absorbent surface by means of a continuous film of paraffin-resistant adhesive, and then impregnating said absorbent surface with paraffin.
10. 2. The method which consists in coating at least one side of a sheet of paper with a paraffin-resisting dry colloid mixed with a tempering agent, printing on the surface so coated, pasting the reverse side of said sheet to a paraffin-absorbent surface by means of a continuous film of paraffin-resisting adhesive, and then impregnating said absorbent surface with paraffin.
15. 3. The method which consists in coating at least one side of a sheet of paper with glue and glycerine, substantially as described, printing on the coated surface, pasting the reverse side of the sheet to an absorbent surface, and saturating said absorbent surface with paraffin.
20. 4. The method of labeling a B-battery box and rendering said box impervious to moisture without impairing the appearance of the label, which consists in treating a surface of a sheet of paper with glue and glycerine, printing on said treated surface, pasting the reverse side of said sheet to an absorbent box by means of a paraffin-resisting glue, and then saturating said box with paraffin.
25. 5. The method of labeling a B-battery box

and of rendering said box impervious to moisture without impairing the appearance 40 of the label, which consists in treating a surface of a sheet of paper with a water solution of about 6% of sizing glue and about 3% of glycerine, drying to form a continuous film, printing on said film, pasting the 45 reverse side of said sheet to an absorbent B-battery box with a film of box-maker's glue, and immersing the box in smoking-hot paraffin.

6. The steps in the process of surfacing 50 the exterior of a B-battery box with a paraffin-resisting paper label, which comprise coating the exposed surface of the paper with a continuous film of glue containing enough glycerine to render the glue film 55 flexible enough for printing without rupture of the film, printing on the surface of the paper so prepared, and fastening the paper to the exterior of the B-battery box with a continuous film of paraffin-resisting adhesive.

7. A paraffin-absorbent paper box having an adhering surfacing of paraffin-resisting paper and having the remainder of its walls 60 saturated with paraffin.

8. A water-proofed B-battery box having an adherent surfacing of printed paraffin-resisting paper and having the remainder of its walls saturated with paraffin.

9. A B-battery box waterproofed with 70 paraffin and having a printed label pasted thereto with paraffin-resistant glue, said label having a surface film of dried colloid and glycerine, substantially as described.

In testimony whereof I affix my signature.  
HOWARD F. WEISS.